

## UNITED STATES PATENT OFFICE

2,476,999

SOLVATION AND DEPOLYMERIZATION OF  
COAL

Milton Orchin, Pittsburgh, Pa., assignor to the  
United States of America as represented by  
the Secretary of the Interior

No Drawing. Application July 24, 1947,  
Serial No. 763,498

6 Claims. (Cl. 196—14)

(Granted under the act of March 2, 1883, as  
amended April 30, 1928; 370 O. G. 757)

1

The invention herein described and claimed may be manufactured and used by or for the Government of the United States of America for governmental purposes without the payment of any royalties thereon or therefor.

This invention relates to the conversion of solid carbonaceous materials, such as bituminous and subbituminous coals, lignites, peat and the like, to liquid products of enhanced value and utility. When such materials are treated in accordance with the invention the primary products are extracts containing little or no ash and which are suitable for direct use as fuels or for use as raw materials for the production of industrial products such as carbon black. Such extracts of low ash content likewise may be used in hydrogenation processes for the production of synthetic liquid fuels corresponding to gasoline, kerosene, Diesel fuels and the like from petroleum sources. Because of the highly aromatic character of the hydrogenation products of such extracts this process provides a means for greatly increasing the potential supply of benzene, toluene and related compounds.

It is an object of my invention to secure the solution of solid carbonizable fuels under the mildest possible conditions whereby secondary reactions will be minimized. A further object of the invention is the improvement of hydrogenation of coal and the like as an extract utilizing for the vehicle selected liquid fractions produced by the hydrogenation of such extracts. Other objects will be apparent from the following description.

A number of processes are known for the extraction of solid pyrobituminous materials such as coal, lignite, peat and the like. In general, all of these processes involve the use as the treating vehicle of mixtures comprising phenols and tetrahydronaphthalene as described, for example, in Pott and Broche Patent 2,147,753 and Pier and Donath Patent 2,215,190. In these prior art methods the ratio of hydrocarbon to phenols in the solvent mixture is customarily about 4:1.

I have found that greatly improved yields of soluble materials can be secured by the use as the solvent vehicle of dicyclic hydro-aromatic compounds containing a phenolic hydroxyl group. Examples of such compounds which are particularly effective are ortho- and para-cyclohexylphenol and tetrahydronaphthols, such as 1,2,3,4-tetrahydro-5-hydroxynaphthalene.

These solvents normally are employed in about equal parts by weight with the solid carbonizable fuel being extracted, that is a ratio of from 1:1 to

3:2. Under some conditions of operations however the amount of solvent may be increased, although in general it is not necessary or desirable to exceed a ratio of about 4:1.

5 The extraction is carried out using finely ground or comminuted coal, lignite and the like with the solvent in the desired ratio, under pressures of about 500 pounds per square inch and at temperatures of about 400° C. While the pressure may be higher or lower than 500 pounds per square inch, normally it should not exceed about 1500 pounds per square inch. Temperatures may vary from about 250° C. to as high as 450° C., although for typical American bituminous coals it is preferred to operate at approximately 400° C. The operating temperature, in any event, should not exceed that at which there is noticeable pyrolysis of the coal, etc., to be extracted.

20 This process may be carried out as a batch type operation or in continuous or semicontinuous manner as desired. Either a neutral or reducing atmosphere may be maintained during the extraction. Under my preferred conditions there is no substantial hydrogenation of the extract.

25 28 the consumption of hydrogen representing from 1-2% by weight of the solid material being extracted.

It is not necessary to use substantially pure compounds in this class. Quite satisfactory results may be secured from crude compounds and mixtures, of course, will give equally desirable results. Thus, mixtures of ortho- and paracyclohexylphenol are suitable for the process, as are mixtures of the tetrahydrohydroxynaphthalenes. 35 The high boiling tar acid fractions from the hydrogenation of certain coals afford a suitable source from which may be conveniently prepared crude mixtures of these novel solvents which may be used without further separation and/or purification.

40 Following the pressure extraction, the solid residual matter is separated from the extract by filtration or centrifuging. The separated solids consist for the most part of the mineral matter, or ash, of the coal or the like starting material, together with unconverted or unextracted starting material. The separation may be effected with or without dilution with the same or other solvents. Such diluents, however, should be

45 50 chemically similar to the initial solvents, preferably containing a phenolic hydroxyl group in the molecule, as I have found that benzene and similar non-polar aromatic compounds are likely to precipitate some of the extracted material. 55 Such precipitates, particularly when admixed

with ash and unconverted coal, are extremely resistant to solvents, and thus lower the liquefaction yield.

The following examples will further and more specifically illustrate the nature of my invention and the manner in which the same may be carried out in practice, but it should be understood that the invention is not limited to said examples.

*Example I*

A Bruceton bituminous coal from the Pittsburgh bed was ground to pass 90% through a 100 mesh screen. This coal had the following analysis:

| Proximate analysis: | Percent by weight |
|---------------------|-------------------|
| Moisture            | 2.1               |
| Volatile matter     | 36.0              |
| Fixed carbon        | 54.7              |
| Ash                 | 7.2               |
| Ultimate analysis:  |                   |
| Hydrogen            | 5.2               |
| Carbon              | 75.5              |
| Nitrogen            | 1.5               |
| Sulfur              | 1.5               |
| Oxygen              | 9.1               |
| Ash                 | 7.2               |

One part of the ground coal was admixed with four parts by weight of o-cyclohexylphenol and charged to a stainless steel autoclave containing hydrogen at one atmospheric pressure. The sealed vessel and contents were heated to 400° C. while being rotated to agitate the contents. The pressure, due to the vapors of the solvent and any permanent gases present, rose to about 500 pounds per square inch. After thirty minutes of treatment the contents of the autoclave were discharged and centrifuged to separate extract from the mineral residue (ash) and unconverted coal constituents. The percentage of extraction was determined as 81.6 calculated according to the following formula:

$$\text{percentage extraction} = 100 - \frac{\text{weight of residue}(100 - \text{per cent ash in residue})}{\text{weight of dry, ash-free coal}}$$

When the same coal is extracted under comparable conditions with a solvent comprising naphthalene, phenol and tetralin (2:1:2) the percentage of extraction was 51.3, while with tetralin alone the percentage was 49.4.

*Example II*

The autoclave was charged with a sample of the same coal used in Example I, admixed with o-cyclohexylphenol in the same proportion, but the treatment was continued for one hour. There was a slight increase in the yield of extracted material, the percentage of extraction calculated as in Example I being 82.8. Substantially the same yield was also obtained upon an increase in time to ninety minutes.

*Example III*

The autoclave was charged with a mixture of 1,2,3,4-tetrahydro - 5 - hydroxynaphthalene and the Bruceton coal used in Example I, in the ratio 4:1 and heated to 400° C. for 30 minutes under an initial hydrogen pressure of 1 atmosphere. The extraction products were separated by centrifuging as described above. The yield was 88.0%.

After separation of the solid residue from the

extract, the latter may be treated by distillation or any other conventional process for recovery of the solvent and the semi-solid extract, the former being reused for extraction of further quantities of the solid carbonizable fuels. The resulting semi-solid material may be utilized in various ways not forming part of the present invention.

The solutions obtained according to this invention are quite stable. A sample of the extract in o-cyclohexylphenol was exposed to air at 45° C. for nineteen days without significant change in appearance or properties. The expressions "solution," "extract" and the like used herein are intended to describe the liquid product from no material can be separated by further filtration or centrifuging. Microscopic examination at 400 magnification indicates substantial absence of solid particles. It is possible, however, that there is actually a form of colloidal dispersion rather than true "solution." Accordingly it will be understood that my invention is not intended to be limited to any particular theory as to the mechanism of the action whereby a substantial proportion of the coal substance is extracted in soluble form.

According to the patent statutes, I have set forth the principles and mode of operation of my invention and have described what I believe to represent its best embodiment. I desire it to be understood, however, that within the scope of the appended claims the invention may be practiced otherwise than as specifically described herein.

35 I claim:

1. A process for the solvation and depolymerization of solid carbonizable fuel for the production of extracts therefrom which comprises treating said fuel with at least an equal weight of a liquid 40 dicyclic hydroaromatic compound containing at least one phenolic hydroxyl group in an atmosphere rich in hydrogen at a temperature of from about 300° C. to about 415° C. and at a pressure corresponding to the vapor pressure of said compound at said temperature and thereafter separating the resulting extract from solid residues.

2. In a process for the preparation of liquid products from solid carbonizable fuel, the improvement which comprises treating the fuel with 50 a liquid dicyclic hydroaromatic compound containing at least one phenolic hydroxyl group in the presence of hydrogen at superatmospheric pressures and at elevated temperatures not in excess of those at which pyrolytic conversion of the fuel will occur.

3. A process for the production of extracts of coals, lignite, peat and the like solid fuel comprising comminuting said fuel, admixing therewith a liquid dicyclic hydroaromatic compound containing at least one phenolic hydroxyl group, heating said mixture to a temperature of about 400° C. in an atmosphere of hydrogen under a pressure corresponding to the vapor pressure of said liquid at said temperature and thereafter separating the extract from the insoluble residue of said fuel at reduced temperatures and pressures.

4. A process for the production of extracts from bituminous coal which comprises treating said coal with at least an equal weight of a solvent 70 composed essentially of ortho-cyclohexylphenol in an atmosphere of hydrogen at a temperature of about 400° C. and under a pressure not in excess of about 1500 pounds per square inch, separating the resulting extract from ash and other solid residues at substantially reduced pressures

and temperatures, recovering at least a major portion of the solvent from said extract and returning recovered solvent to the process for treatment of further quantities of coal therein.

5. A process for the production of extracts from bituminous coal which comprises treating said coal with at least an equal weight of a solvent composed essentially of para-cyclohexylphenol in an atmosphere of hydrogen at a temperature of about 400° C. and under a pressure not in excess of about 1500 pounds per square inch, separating the resulting extract from ash and other solid residues at substantially reduced temperatures and pressures, recovering at least a major portion of the solvent from said extract and returning recovered solvent to the process for treatment of further quantities of coal therein.

6. A process for the production of extracts from bituminous coal which comprises treating said coal with at least an equal weight of a solvent composed essentially of 1,2,3,4-tetrahydro-5-hydroxynaphthalene in the presence of hydrogen at a temperature of about 400° C. and under a pressure not in excess of about 1500 pounds per square inch, and separating the resulting extract

from ash and other solid residues at substantially reduced temperatures and pressures.

MILTON ORCHIN.

#### REFERENCES CITED

The following references are of record in the file of this patent:

#### UNITED STATES PATENTS

| 10 | Number    | Name                | Date          |
|----|-----------|---------------------|---------------|
|    | 1,822,349 | Jannek et al. _____ | Sept. 8, 1931 |
|    | 2,147,753 | Pott et al. _____   | Feb. 21, 1939 |

#### FOREIGN PATENTS

| 15 | Number  | Country             | Date         |
|----|---------|---------------------|--------------|
|    | 234,564 | Great Britain _____ | June 4, 1925 |

#### OTHER REFERENCES

Bull. soc. chim. Belg., vol. 43, pages 382-391 (1934) by Gillet et al., abstracted in Chem. Abstracts 29, page 16087.

Ellis, "Hydrogenation of Organic Substances," 3rd edition, page 236, published Nov. 1930, Van Nostrand & Co., New York.